

Patented Feb. 2, 1926.

1,571,662

# UNITED STATES PATENT OFFICE.

ANDREW A. DUNHAM, OF BAINBRIDGE, NEW YORK, ASSIGNOR TO THE CASEIN MANUFACTURING COMPANY, OF NEW YORK, N. Y., A CORPORATION OF VERMONT.

## CASEIN WATERPROOF GLUE.

No Drawing.

Application filed April 28, 1924. Serial No. 709,688.

To all whom it may concern:

Be it known that I, ANDREW A. DUNHAM, a citizen of the United States, and resident of Bainbridge, Chenango County, State of 5 New York, have invented certain new and useful Improvements in Casein Waterproof Glues, of which the following is a specification.

This invention has for its object an 10 improvement in casein water-proof glues which, when applied to wood, will prevent or minimize discoloration of the same.

The so-called water-proof casein glues, as 15 is well known to those skilled in the art, contain as their principal ingredients casein and one or more of the alkaline earth oxids or hydroxids, the latter being used in considerable excess above the amount necessary to dissolve the casein. The oxid or hydroxid 20 of calcium is almost universally employed because it is least expensive and gives the best results. These glues, while possessing many advantages, possess the disadvantage of discoloring the surfaces of certain kinds 25 of wood to a great degree, it being almost impossible to use them commercially for gluing mahogany, walnut and other woods of this class, especially in the form of thin veneers. The discoloring or stain penetrates 30 the pores of the wood to such an extent that the resulting product is unavailable for use in making articles in which the veneer is exposed to view.

I have found that the staining or discoloring of the wood is, to a very great degree, 35 prevented by having finely ground wood fibre present in the glue. Although I do not claim that I can completely prevent discoloration, I can, by the means indicated, 40 arrest, to a considerable extent, the tendency of the stain to penetrate thin veneers and appear on the outer surface. I prefer to use wood-flour made from the hard woods such as birch, beech and maple, although 45 wood-flour made from other kinds of woods may be used if desired. I prefer to use from 5% to 20% by weight of wood-flour to from 95% to 80% of casein glue; I find that within these proportions there is little 50 or no loss of strength in the glued joint, but on the contrary in most cases I obtain added strength, probably because of the cohesion of the small particles of wood-flour with each other and with the interior surfaces of the pores of the wood to be glued.

While I may use less than 5% of wood-flour, I find that with this proportion the tendency of the stain to penetrate to the outer surface of the wood is more pronounced; and while I may use more than 20% 60 of wood-flour, I find that with this proportion the glue is apt to lose its spreading qualities and that there is a decrease of strength in the resulting glued joint. For convenience of manufacture, I prefer to mix 65 my wood-flour with the casein at the same time that the alkaline earth hydroxide and other chemicals are mixed therewith.

The following examples will illustrate my 70 invention:

### Example 1.

95 lbs. by weight of a casein water-proof glue made up in the proportions, by weight, of 60% casein, 30% lime and 10% sodium carbonate are mixed with 5 lbs. of fine wood-flour of the ordinary commercial grades. This mixture is preferably made dry. The resulting glue base is then ready to be shipped to a veneer mill to be used in gluing 80 wood in the well known manner.

### Example 2.

90 lbs. of the dry casein water-proof glue of the composition specified in example 1 85 are thoroughly mixed with 10 lbs. of ordinary commercial finely ground wood-flour. The method of dissolving and applying this glue is the usual one well known to the art.

### Example 3.

80 lbs. of the casein water-proof glue of the composition specified under example 1 are mixed with 20 lbs. of ordinary commercial finely ground wood-flour. After thorough 95 mixing, the resulting material is ready to pack and ship for use in the usual manner.

As casein water-proof glue is marketed in the form of a mixture of the dry ingredients, water being added just before the glue is to be applied to the surfaces to be united, the designation "glue" is generally employed in the art to designate not only the dry mixture, but also the material when it has been made ready to spread by the addition of water, and the material after it has set to form the joint. It is in this customary sense that I desire the designation "glue", used in the claim, to be understood.

When I speak in my claim of a casein 110

water-proof glue I do not limit myself to any particular composition of a glue of this type. Such a glue may, if desired, contain in addition to the principal ingredients al-  
5 ready referred to other casein solvents such as carbonates, bicarbonates, phosphates, sul-  
fites, silicates, fluorides and the like, and the amounts of the chemical or chemicals used with casein to make the glue may vary  
10 to a fairly large degree depending upon the quality of the casein used as well as the particular work for which the glue is to

be employed, for instance, for the gluing of thick blocks of wood the composition of the glue may have to be different from that 15 which is to be used for the gluing of veneer.

I claim:

As a composition of matter, a casein water-proof glue having incorporated therewith from 5% to 20% by weight of wood- 20 flour substantially as and for the purpose described.

ANDREW A. DUNHAM.